

## UNITED STATES PATENT OFFICE

2,251,266

## MAGNESIUM ALLOY

Arthur Burkhardt, Berlin-Lichterfelde, Richard Knabe, Berlin-Zehlendorf, and Karl Riederer, Munich, Germany, assignors to Georg Von Giesche's Erben, Breslau, Germany, a corporation of Germany

No Drawing. Application November 9, 1939, Serial No. 303,610. In Germany December 16, 1938

4 Claims. (Cl. 75—168)

Our invention relates to a magnesium alloy, and more especially to an alloy of the type described in U. S. Patent 2,159,964, for "Magnesium alloy," patented May 30, 1939.

In this patent, a magnesium alloy has been described that contains 2 to 6% bismuth, 0.5 to 3% cadmium, 1 to 5% aluminium, and 1 to 3.5% zinc. The remainder is substantially all magnesium. The phrase "substantially all magnesium" is intended to include magnesium and magnesium with minor amounts of customary impurities and auxiliaries. Such auxiliary alloying elements are, for instance, 0.1 to 2% each of manganese, calcium, silicon, or one of the metals of the iron group (iron, nickel, and cobalt) separately or collectively. Such and other auxiliaries are usual in magnesium alloys and they do not influence the characteristic properties of our novel alloys.

Preferably, the alloy described in the said patent contains 4 to 5% bismuth, about 2% cadmium, 2 to 4% aluminium, and about 3% zinc, the remainder being substantially all magnesium, as defined above.

The said alloy possesses satisfactory resistance to corrosion and, first and foremost, high mechanical properties.

It is an object of our invention to improve an alloy of the type aforesaid, especially with a view to increasing its ductility.

To this end, we add to the said alloy 0.2 to 4% titanium.

The magnesium alloy according to our invention is consequently characterised by a content of 2 to 6% bismuth, 0.5 to 3% cadmium, 1 to 5% aluminium, 1 to 3.5% zinc, about 0.2 to 4% titanium, remainder substantially all magnesium.

Preferably, the alloy according to our invention contains 4 to 5% bismuth, about 2% cadmium, 2 to 4% aluminium, about 3% zinc, about 0.2 to 4% titanium, remainder substantially all magnesium.

The titanium-containing magnesium alloys according to the invention compare favorably with the alloys according to the said U. S. patent in that their ductility is improved, as demonstrated by higher values of elongation and reduction of area. Thus, with a tensile strength of about 40 to 45 kg. per sq. mm., which is equal to that of the alloys according to the said U. S. patent, their elongation is 14 to 8%, and their reduction of area is as high as about 25%.

The zinc content of the alloys according to the invention may be higher than the upper limit of 3.5%, as indicated above, and may be up to 7%. In this manner, we provide mag-

nesium alloys of high tensile strength and particularly high ductility.

By way of example, an alloy according to the invention may have the following composition: 2 to 6% bismuth, 0.5 to 3% cadmium, 1 to 5% aluminium, 1 to 7% zinc, about 0.2 to 4% titanium, remainder substantially all magnesium.

By increasing the content of zinc up to 7%, as described, we provide alloys whose tensile strength is 34 to 36 kg. per sq. mm. and whose elongation is about 22 to 24%. Due to the content of about 0.2 to 4% titanium, the ultimate strength of the alloys is still further increased.

In the following tabulation, some more examples of alloys according to our invention are given, it being understood that for all alloys in the tabulation the remainder is substantially all magnesium as defined above, that is, magnesium with or without the aforesaid minor amounts of customary impurities and/or auxiliaries.

## Examples

| No. | No. | Content of constituents, per cent |    |    |     |     |
|-----|-----|-----------------------------------|----|----|-----|-----|
|     |     | Al                                | Bi | Cd | Zn  | Ti  |
| 1   |     | 5                                 | 4  | 2  | 3   | 0.2 |
| 2   |     | 5                                 | 4  | 2  | 3   | 1   |
| 3   |     | 5                                 | 4  | 2  | 3   | 3   |
| 4   |     | 5                                 | 2  | 3  | 3   | 0.3 |
| 5   |     | 5                                 | 2  | 3  | 3   | 1.5 |
| 6   |     | 4                                 | 4  | 2  | 2   | 0.5 |
| 7   |     | 5                                 | 4  | 2  | 4   | 0.5 |
| 8   |     | 5                                 | 4  | 2  | 5   | 2   |
| 9   |     | 4                                 | 4  | 2  | 6.5 | 1.5 |
| 10  |     | 5                                 | 4  | 2  | 7   | 1   |

We claim:

1. A magnesium alloy containing 2 to 6% bismuth, 0.5 to 3% cadmium, 1 to 5% aluminium, 1 to 3.5% zinc, about 0.2 to 4% titanium, the remainder substantially all magnesium.

2. A magnesium alloy containing 4 to 5% bismuth, about 2% cadmium, 2 to 4% aluminium, about 3% zinc, about 0.2 to 4% titanium, the remainder substantially all magnesium.

3. A magnesium alloy containing 2 to 6% bismuth, 0.5 to 3% cadmium, 1 to 5% aluminium, 1 to 7% zinc, about 0.2 to 4% titanium, the remainder substantially all magnesium.

4. A magnesium alloy containing 2 to 6% bismuth, 0.5 to 3% cadmium, 1 to 5% aluminium, more than 3.5 to 7% zinc, about 0.2 to 4% titanium, the remainder substantially all magnesium.

ARTHUR BURKHARDT.  
RICHARD KNABE.  
KARL RIEDERER.